

## UNITED STATES PATENT OFFICE

EDWARD BEGLINGER AND JOHN M. GAHAGAN, OF MADISON, WISCONSIN, DEDICATED  
TO THE FREE USE OF THE GOVERNMENT AND THE PEOPLE OF THE UNITED STATES  
OF AMERICA

## METAL FASTENING AND PROCESS FOR MANUFACTURING THE SAME

No Drawing.

Application filed August 22, 1931. Serial No. 558,847.

(GRANTED UNDER THE ACT OF MARCH 3, 1883, AS AMENDED APRIL 30, 1928; 370 O. G. 757)

This application is made under the act of March 3, 1883, as amended by the act of April 30, 1928, and the invention herein described, if patented, may be manufactured and used by or for the Government, for governmental purposes, without payment to us of any royalty thereon.

We hereby dedicate the invention herein described to the free use of the public to take effect upon the granting of a patent to us.

Our invention consists of a microscopic pitting or etching of metal fastenings to such an extent as to cover their surfaces with minute indentations, the purpose of the pitting being to promote better contact between the fastening and the wood and hence increase the resistance to withdrawal. This is very desirable since the resistance to withdrawal of a fastening from wood or other material depends largely upon the nature and extent of this area of contact.

To the unaided eye the pitted surface we have invented appears the same as the original in that there is no apparent roughening. In fact, the surface may be considered smoother than the original, which, as a rule, is considerably roughened in manufacture.

Treatments heretofore proposed for increasing the holding power of nails and other fastenings consist either of a surface coating or a grossly roughened surface produced either by mechanical or chemical action. The coatings have the distinct disadvantage that they may be removed in handling or driving, or their effectiveness may be otherwise lost through disintegration with time. The roughened surfaces that are produced by sand blasting, barbing, or by gross pitting of any sort, tend to reduce the area and intimacy of contact between the fastening and the wood fibers, which is so essential to high holding power and which is fully developed by the microscopically pitted surface that we have invented.

The mechanism of the process used in obtaining this surface pitting effect is extremely simple. It is as follows:

(1) The fastening is subjected to the ac-

tion of water solutions of ferric chloride in which is present a salt of some other metal, but more specifically with the chloride salt of a metal falling below iron in the electrochemical series; (2) the fastening is withdrawn from the solution and allowed to dry in a warm atmosphere; (3) the fastening is subjected to an atmosphere whose temperature and humidity are under control. Experience has shown satisfactory results at temperatures of about 100° C. and humidities of about 80 per cent; (4) the fastening is removed from this atmosphere and immediately immersed in boiling water to fix resulting oxides adhering to the surface.

The following is a specific example of a treatment which has given excellent results for a ferrous metal fastening:

The fastening to be treated is immersed for a period of five to six seconds in 100 c. c. of a 2 per cent water solution of ferric chloride containing 2 g. mercuric chloride. It is then withdrawn and allowed to remain in a warm atmosphere for 10 minutes so that evaporation of the greater part of the solution may be effected. The fastening is next placed in an atmosphere where the temperature is 100° C., and the relative humidity 75 to 80 per cent. After a period of 60 minutes in this atmosphere, the fastening is removed and immediately immersed in boiling water for five minutes, removed and allowed to dry at atmospheric temperature. The loosely adhering black oxide may be removed by buffing in dry sawdust or by other suitable means. The addition of methyl alcohol to a solution of the above described type has a beneficial effect in some instances but is not considered as essential in this processing.

It is obvious that for different materials to be pitted, the treating solution and the conditions of the processing may be so modified as to effect the desired surface pitting.

A number of tests made on wire nails and staples, with surfaces microscopically pitted or etched, as above described, gave decidedly higher values for resistance to withdrawal than were obtained with similar fastenings having plain, cement-coated, or grossly

roughened surfaces. The same superiority was shown by the microscopically pitted fasteners whether they were pulled immediately after driving or after a lapse of approximately one year.

Having fully described our discovery, we claim as our invention:

1. An improvement in the process of manufacturing ferrous metal fastenings comprising subjecting such fastenings to the action of a water solution containing 2 per cent ferric chloride and 2 per cent mercuric chloride.
2. An improvement in the process of manufacturing ferrous metal fastenings comprising immersing such fastenings in a water solution containing 2 per cent ferric chloride and 2 per cent of a salt of a metal falling below iron in the electro-chemical series, withdrawing said fastenings from the solution and allowing them to dry in a warm atmosphere, then subjecting the fastenings to a temperature of approximately 100° C. and a humidity of approximately 80 per cent, removing the fastenings from said temperature and immediately immersing them in boiling water to fix the resulting iron oxides adhering to the surfaces.
3. An improvement in the process of manufacturing ferrous metal fastenings, comprising immersing such fastenings for a period of 6 seconds in a 2 per cent water solution of ferric chloride, containing 2 per cent mercuric chloride, withdrawing said fastenings from the solution and allowing them to dry in a warm atmosphere for 10 minutes, then subjecting the fastenings to a temperature of 100° C. with a relative humidity of 80 per cent for a period of 60 minutes, removing the fastenings from the said temperature and immediately immersing them in boiling water for 5 minutes and drying them at atmospheric temperature.

EDWARD BEGLINGER.  
JOHN M. GAHAGAN.

50

55

60

65